

## UNITED STATES PATENT OFFICE

2,395,996

## PRODUCTION OF A ROAD JOINT SEALING COMPOSITION

John T. Doyle, deceased, late of Anne Arundel County, Md., by Mary H. Doyle, administratrix, Baltimore, Md.

No Drawing. Application May 28, 1942,  
Serial No. 444,935

1 Claim. (Cl. 196—74)

The invention relates to the construction of concrete and similar pavements which in order to prevent or reduce cracking due to expansion and contraction with changes of temperature are cast in sections which are spaced in correspondence with the degree of contraction and expansion expected. These spaces or joints between the sections are bridged at a level below the road surface by load transfer members cast in the concrete and are usually filled below the surface with a precast asphaltic or other resilient filler which is placed in position before pouring the concrete. The joints may extend longitudinally of the roadway as well as transversely.

An extremely important consideration is the exclusion of moisture the entrance of which into the joints and through the joints into the subgrade causes disruption due to alternate freezing and thawing, hence the necessity for the moisture proof seal, which is the subject of the invention.

In the process of construction the precast filler plates or such filler as may be employed are set on the lines of the joints, each in upright position, with its top edge below the road surface. This leaves a rabbet or groove which in cross section is customarily about three quarters of an inch by three quarters of an inch or thereabouts, overlying the filler at the top of the joint. This groove or rabbet is subject to contraction and expansion transversely of its length as the concrete sections or slabs between which it is located expand and contract.

When the pavement is set these grooves or rabbets are filled with a sealing compound the main purpose of which is to prevent the entrance of moisture into the joints and through the joints into the subgrade. A purpose is also of importance is to fill the joints substantially flush with the road surface and thus bridge the joints preventing the bumping of the tires in passing the joints or reducing it to the minimum.

The problem presented is different from that involved in the sealing of road cracks, and the compositions suitable for the latter purpose are not suitable for use in the sealing of the joints and likewise the present composition in the preferred form is not suitable to the sealing of road cracks as it sets or partially sets so promptly that it cannot be satisfactorily introduced into openings of the width which such cracks normally assume.

In the mid-temperate zone to which the bulk of the area of the United States proper may be said to belong, there is an annual variation of

road surface temperature of over 100° F., a variation of 130° F. being close to the average.

A satisfactory road sealing compound must be capable of low cost production, and easy of application and should meet these temperature conditions and continue over a long period to be effective in the exclusion of water and in the bridging of the groove in such a manner as to substantially eliminate bumping of the tires in crossing the joints. Various bituminous compounds and mixtures of rubber, asphalt, tar and other plastic substances have been employed with notable absence of satisfactory results. So far as can be ascertained no satisfactory composition for this purpose which can be produced at a figure commensurate with a reasonable cost of construction has yet been produced or offered to the builders of concrete and similar pavements.

The difficulties encountered include primarily the tendency of the sealing composition to harden and crack in cold weather when the concrete sections or slabs contract and the grooves or rabbets expand and these cracks form leaks which admit water to the joints and to the subgrade. A further difficulty is the tendency of the sealing material to liquefy at the higher road temperatures so that it escapes from the joints both by leakage and by distribution over the road surface due to partial adhesion to vehicle tires. The majority of these joint sealing compositions also lack the adhesiveness necessary to cause them to remain attached to the side walls of the grooves in cold weather and also lack the flexibility and elasticity or ductility at low temperatures necessary to permit them to expand with the expansion of the groove which causes cracking and leakage as already pointed out. The prior compositions not only lack the necessary properties of low temperature elasticity or ductility and low temperature adhesiveness but are so extremely fluid or ductile at the higher road temperature that they escape from the joint by leakage and adhesion to the tires of passing vehicles. There is also a tendency of the prior compositions due to alternate heating and cooling to form hard protuberances which cause highly objectionable bumping of the tires.

The object of the present invention is the production and application of a concrete road joint sealing composition whereby the difficulties above recited and other difficulties which occur in the manufacture and use of the previously known compositions for this purpose are overcome.

The composition has been thoroughly tested

under the circumstances and conditions encountered in actual practice and is known to meet the requirements more fully and completely than does any previously known road joint sealing composition. Namely this composition retains a sufficient degree of flexibility and elasticity at low temperatures to prevent cracking and is sufficiently solid and non-fluid or free from excess ductility at the highest road temperatures to prevent escape from the joint and to prevent loss by smearing on the pavement surface and on the tires of passing vehicles. It is also of importance that this composition affords satisfactory support for the tires in passing the joints and does not form protuberances which would cause bumping of the tires, nor does it when properly applied become separated from the sides or side walls of the grooves, particularly in cold weather, forming cracks which admit water. It also has satisfactory sealing properties at medium temperatures.

In the practice of the invention in what is regarded as the preferred form, a reasonable degree of variation and substitution being contemplated, the disclosure serving mainly as an example of the successful practice of the invention, the sealing composition is manufactured by blending a material having the properties and composition of steam refined asphalt made from Texas crude or substantially such properties, the same being of approximately 50-60 penetration by the standard penetration test which is understood to mean 50 to 60 one hundredths of a centimeter penetration by a standard test needle under 100 grams pressure applied for a period of five seconds at a temperature of 77° F. A blend which has been successful in the practice of the invention comprises 70% asphalt of the quality above described and 30% by volume of an intermediate or flux oil.

The above description is intended to define an asphalt of high ductile qualities containing little or no paraffin and the minimum of sulphur, both of which constituents are regarded as undesirable.

Steam refining is mentioned as giving the desired result, the possibility of obtaining similar conditions and results and an asphalt of similar qualities by other methods of refining being recognized, the method of producing this constituent not being a feature of the invention.

The proportions stated and the quality of the thinning or intermediate oil are also subject to such variation as does not forfeit the essential properties of the resulting composition. The intermediate or flux oil used is preferably free or substantially free of sulphur and paraffin.

An intermediate or flux oil which has proved satisfactory for this purpose may be identified as follows according to generally recognized standard tests.

American Petroleum Institute hydrometer @ 60°, 13°-14°.

Flash point, C. O. C. (Cleveland open cup), 480° F. 65 Furool viscosity, @ 210° F. 45 seconds.

Float test, @ 150° F. 16 seconds.

While neutral solids in finely divided form and other ingredients may be added such additions are regarded as unnecessary and generally undesirable in the light of the information at hand.

The description of the intermediate or flux oil or thinning agent will serve to identify an oil which is found to be satisfactory for this purpose, the possibility of variation and substitution

to meet the conditions encountered having been mentioned.

In the practice of the process whereby the desired result has been attained the materials in suitable proportion, for example 70 parts asphalt to 30 parts oil thus mixed are blown with air to a softening point designated as approximately 135° F., a reasonable degree of variation above and below this point being regarded as feasible and a variation from 130° F. to 140° F. having been ascertained as not interfering with the useful result attained. The temperature of the softening point or melting point of the blend is raised by blowing as described, and the ductility at high temperatures is reduced. Mixing as described gives an increased ductility and penetration at low temperature which is retained to a satisfactory degree after blowing. The properties of the combined materials are thus determined by mixing and blowing, the result being a satisfactory joint sealing compound. The term "softening point" thus employed has reference to a standard test prescribed by the American Society for the Testing of Materials and thus identified. Blowing is understood to effect partial oxidation. A blowing temperature of 485° F. has been found satisfactory. Compensating variations of time, air supply and temperature may be practiced.

The resulting material when used as a concrete road joint sealing compound conforms to the requirements above recited. This composition may be characterized and identified according to the practice in selecting and determining petroleum and similar plastics as follows:

35 Melting point (ring and ball test), approximately 135° F.

Penetration by standard test @ 32° F., 200 grams pressure standard test needle duration 60 seconds, minimum 20, approximately normal variation 20 to 30 (unit of penetration being  $\frac{1}{100}$  centimeter).

Penetration, @ 77° F., 100 grams pressure standard test needle, duration 5 seconds, approximately 50 to 60 units of penetration.

40 45 Penetration, 115° F., 50 grams pressure, 5 seconds maximum, approximately 175 units of penetration by standard test needle.

Ductility @ 77° F. stretching at rate of 5 centimeters per minute, approximate stretch 80 to 50 100 without cracking.

Ductility, @ 32° F. stretch at rate of 0.25 centimeter per minute without cracking approximately 4.

Flash point, approximately 500° F.

55 60 The ductilities referred to are determined by and stated in terms of test D 113-39, American Society for Testing Materials.

Solubility in carbon disulphide, 99% minimum.

The foregoing specification identifies the product of the invention in the preferred form from which some relaxation of the requirements or a degree of variation may be permitted. The asphaltic composition of the invention is regarded as unique in the attainment of this standard particularly as to excessive ductility and penetration at low temperatures and a relatively low maximum penetration at high temperatures as stated, which constitute a notable accomplishment in a composition for the sealing of joints of concrete pavements. The other properties stated are given mainly for the purpose of describing the composition in what is at present regarded as the preferred form.

In sealing the joints of concrete roads in accordance with the preferred practice of the in-

vention the sides or side walls of the groove or rabbet at the top of the joint are preferably first coated with an asphaltic paint following which the grooves or rabbets are filled with the joint sealing composition of the invention, for which purpose the sealing composition is liquefied by heating, the temperature being preferably from 325° to 340° F., 350° being regarded as the maximum temperature to which it can be heated without probability of deterioration. Other priming fluids may be employed.

This sealing composition is of an asphaltic nature having the properties above identified and imparted to it by the treatment, above defined.

A satisfactory material for priming or coating the walls of the grooves or rabbets to improve the adhesion of the composition may be made by combining a liquid petroleum product substantially of the nature of naphtha or the equivalent or other suitable thinning agent with a 50-60 steam refined asphalt or asphaltic composition of the properties previously defined under this heading, the manner and source of production being immaterial. This mixture or paint may consist of 70% naphtha or the equivalent to 30% asphalt which is preferably of the quality used in the sealing composition the proportions and constituents being subject to some variation. Other priming may be used.

The terms "Texas crude petroleum," "steam refined asphalt," "naphtha," "intermediate oils" and the like are used to identify materials of satisfactory qualities and properties without regard to the source or the manner of production or intended limitation as to such source or manner of production.

I have thus described a road sealing composition and method of making the same as an example of the practice of the invention in con-

nnection with the problem involved, the description being specific and in detail in order that the manner of practicing, applying and using the invention may be fully understood. However, the composition and the method described are subject to variation in the light of a full knowledge of the nature of the materials and problems involved and the specific terms are used in a descriptive rather than a limiting sense, the scope of the invention being defined in the claim.

What is claimed as new and desired to be secured by Letters Patent is:

The method of making a sealing composition for concrete road joints, which consists of blending approximately 70% asphalt, the same having a penetration of 50-60 at 77° F., the said asphalt being combined with 30% by volume of an intermediate oil containing practically no paraffin, and practically no sulphur, the said oil having a flash point of approximately, 480° F., a Furol viscosity of approximately, 45 seconds at 210° F., and a float test at 150° F. of approximately 16 seconds, thereafter blowing with air at a temperature of approximately 485° F. for a period sufficient such that the resulting material will have a softening point by the ring and ball test of approximately, 135° F. penetration at 32° F., approximately, 20 to 30, under a thrust of 200 grams for 60 seconds, penetration at 77° F., approximately 50-60, under a thrust of 100 grams for 5 seconds, and a penetration at 115° F., of approximately 175, under a thrust of 50 grams for 5 seconds, a ductility at 77° F., of approximately 80 to 100, a ductility at 32° F., approximately 4, and flash point of approximately 500° F.

MARY H. DOYLE,  
*Administratrix of the Estate of John T. Doyle,  
Deceased.*